

# UNITED STATES PATENT OFFICE.

FREDERIC LEWIS NATHAN AND WILLIAM RINTOUL, OF STEVENSTON, AND FRANK BAKER, DECEASED, LATE OF STEVENSTON, SCOTLAND, BY HENRY BAKER, OF ETON, WINDSOR, ENGLAND, ADMINISTRATOR OF SAID FRANK BAKER, ASSIGNEES TO NOBEL'S EXPLOSIVES COMPANY, LIMITED, OF GLASGOW, SCOTLAND.

## GELATINIZED PROPELLENT EXPLOSIVE AND PROCESS OF PREPARING SAME.

1,338,691.

Specification of Letters Patent.

Patented May 4, 1920.

No Drawing. Application filed February 26, 1914, Serial No. 821,338. Renewed October 21, 1918. Serial No. 259,071.

*To all whom it may concern:*

Be it known that Colonel Sir FREDERIC LEWIS NATHAN and WILLIAM RINTOUL, both subjects of the King of Great Britain and 5 Ireland, and residing at Ardeer, Stevenston, Ayrshire, Scotland, and FRANK BAKER, deceased, late of Ardeer, Stevenston, Ayrshire, Scotland, invented a certain new and useful Gelatinized Propellant Explosive and 10 Process of Preparing Same, of which the following is a specification.

This invention relates to gelatinized propellant explosives.

Such explosives at the present day are 15 generally prepared by gelatinizing nitrocellulose, with or without nitroglycerin by a volatile solvent but this has many disadvantages chiefly residing in the slowness of the drying operation adopted for expelling 20 the solvent from the gelatinized mass, in the impairment of the stability of the material due to the heating and in the changes consequent on slow after-drying during storage.

In the course of investigations having for 25 their object to discover improved stabilizers for nitric ester explosives we have found that among the groups of bodies ascertained to be good stabilizers—certain anilids, aromatic-radical-containing substituted carbaminic acid, esters, aromatic-radical-containing partially substituted ureas, and aromatic-radical-containing simple or mixed ethers (see applications Serial No. 771,621, filed June 4, 1913, Patent No. 1,090,642 30 granted March 17, 1914; Serial No. 771,623 filed June 4, 1913, Patent No. 1,090,644 granted March 17, 1914; Serial No. 771,620 filed June 4, 1913, Patent No. 1,090,641 granted March 17, 1914; Serial No. 771,622 35 filed June 4, 1913, Patent No. 1,090,643, granted March 17, 1914)—are a number which are also good gelatinizers for nitrocellulose so that by using them both gelatinization, without the above inconveniences, 40 and stabilization can be obtained.

We have now further found however that satisfactory results can be attained without necessarily using a substance which of itself performs these two functions and that provided 45 certain conditions are complied with a gelatinized propellant explosive can be so obtained which can be prepared without the

inconveniences in working with a volatile solvent and of good chemical and physical stability.

The conditions in question are that in the first place the gelatinizing agent shall be sufficiently soluble in nitroglycerin to remain dissolved in product, secondly that a stabilizing agent must be present which 55 shall be capable of taking up the products of the inevitable slow decomposition of such explosives however carefully prepared and thirdly that these bodies must be such that neither singly nor when present together or 60 when acted upon by the products of slow decomposition do they act to accelerate this 65 decomposition.

It has been found that the neglect of any one of these conditions is sufficient to render 70 the product an unsatisfactory one—segregation and change in both composition and ballistics accompanying insufficient solubility of the gelatinizer in the nitroglycerin; the accelerating effect of the products of 75 slow decomposition upon the further decomposition of the material when they are allowed to remain in contact with the material and not disposed of by a stabilizer being such as to render the material inserviceable and often dangerous and the presence 80 of an unsuitable radical or group in the stabilizing or gelatinizing compounds used or those formed from them with the products of decomposition during storage readily leading to series reduction in the stability of the explosive.

According to this invention therefore gelatinized propellant explosives are prepared 85 from nitrocellulose and nitroglycerin by incorporating with them a gelatinizing agent and a stabilizing agent of the character in question.

In carrying the invention out in one way the following ingredients, namely 40 parts 90 of nitroglycerin, 50 parts of soluble nitrocellulose, 7.5 parts of para-nitro-methylacetanilid (the gelatinizer) and 2.5 parts of ethyl- $\beta$ -naphthyl-ether (the stabilizer) are brought together by the wet suspension 95 method of Lundholm, English Patent No. 10376 of 1889, the gelatinous mass separating from the aqueous suspension of the materials being freed as far as possible 100

from water by pressing and rolling between rollers heated to from 40° C. to 50° C., then gelatinized by rolling at a temperature of from 50° C. to 70° C. and the sheet so obtained cut into flakes or strips or pressed into any desired form by a pressure of several hundred atmospheres applied to it at a temperature of from 50° to 70° C.

This example is one in which the gelatinizer is a body falling within the classes first above referred to as furnishing good gelatinizers but which owing to the presence of an unsuitable group in it is not possessed of satisfactory stabilizing properties and so excluded from use for that purpose, and in this example this is compensated by using a body of another of these classes, an ether, to give the stabilizing effect.

At the same time while the classes of bodies referred to do in this way furnish good gelatinizers a wide variety of other materials sufficiently soluble in nitro-glycerin (say to the extent of about 25% at least at ordinary temperatures) and complying with the other conditions is available of which amyl phthalate, ethyl phthalate, mono-, di- or tri-acetin, and nitro derivatives of aromatic hydrocarbons such as di- and trinitrotoluene are instances.

Again the stabilizer need not fall within the classes first considered provided it satisfies the requirements indicated and preferably is soluble to the extent of not less than 5% in nitroglycerin and phenanthrene (see Spica, *Zeit. f. Schiess- und Sprengstoff-wesen* 1912 p. 129) is an instance of such a body. Our experience has shown us that stabilizers soluble in nitroglycerin tend to increase in solubility in admixture of nitro-glycerin and gelatinizer.

Examples of suitable mixtures are—

(a) 40 parts nitroglycerin, 50 parts soluble nitrocellulose (12.6% nitrogen) 7.5 parts ethyl phthalate as gelatinizer and 2.5 parts ethyl-β-naphthyl ether as stabilizer.

(b) 40 parts nitroglycerin, 50 parts soluble nitrocellulose, 7.5 parts ethyl phthalate and 2.5 parts phenyl-benzyl ether.

(c) 40 parts nitroglycerin, 50 parts soluble nitrocellulose, 7.5 parts para-nitro-methyl acetanilid and 2.5 parts phenanthrene.

Where the wet incorporation method is used and the substances to be employed as gelatinizer and stabilizer are soluble in water it is preferable to use as the suspending liquid a solution of these bodies in water and of such a concentration that the resulting paste will have the desired composition.

We claim:

1. The process which comprises mixing together nitro-cellulose, nitroglycerin, para-nitro-methyl-acetanilid, and a stabilizing substance soluble in the mixture of these ingredients and then gelatinizing the mixture.

2. The process which comprises mixing together nitrocellulose, nitroglycerin, para-nitro-methyl-acetanilid and a stabilizing substance soluble in the mixture of these ingredients, said substance being a readily nitratable aromatic radical containing compound, and then gelatinizing the mixture. 70

3. A propellant explosive comprising a gelatinous admixture of nitrocellulose, nitroglycerin, paranitro-methyl-acetanilid, 75 and a stabilizing substance soluble in the mixture comprising the previously mentioned constituents.

4. A propellant explosive comprising a gelatinous admixture of nitrocellulose, nitroglycerin, a paranitro-methyl-acetanilid, 80 and a stabilizing substance soluble in the mixture comprising the previously mentioned constituents, said substance being a readily nitratable aromatic radical containing compound. 85

5. A propellant explosive comprising a gelatinous admixture of about 50 parts of soluble nitrocellulose, about 40 parts of nitroglycerin, about 7.5 parts of para-nitro-methyl acet-anilid and about 2.5 parts phenanthrene. 90

6. A propellant explosive comprising a gelatinized admixture of soluble nitrocellulose, nitroglycerin and para-methyl-acet-anilid. 95

7. A propellant explosive comprising a gelatinized admixture of soluble nitrocellulose, nitroglycerin, para-nitro-methyl-acet-anilid, and phenanthrene. 100

8. The process which comprises mixing together nitrocellulose, nitro-glycerin, a non-volatile gelatinizing agent sufficiently soluble in the nitro-glycerin to remain dissolved in the mixture, and a stabilizing agent capable of taking up any products of decomposition, and which will not accelerate decomposition in the presence of the other constituents, and then gelatinizing the mixture. 105

9. The process which comprises mixing together nitrocellulose, nitro-glycerin, a non-volatile aromatic gelatinizing compound sufficiently soluble in the nitro-glycerin to remain dissolved in the mixture, and a stabilizing agent capable of taking up any products of decomposition, and which will not accelerate decomposition in the presence of the other constituents, and then gelatinizing the mixture. 115

10. The process which comprises mixing together nitrocellulose, nitro-glycerin, a non-volatile gelatinizing agent sufficiently soluble in the nitro-glycerin to remain dissolved in the mixture, and an aromatic stabilizing compound capable of taking up any products of decomposition, and which will not accelerate decomposition in the presence of the other constituents, and then gelatinizing the mixture. 120

125

125

130

11. The process which comprises mixing together nitrocellulose, nitro-glycerin, a non-volatile aromatic gelatinizing compound sufficiently soluble in the nitro-glycerin to remain dissolved in the mixture, and an aromatic stabilizing compound capable of taking up any products of decomposition, and which will not accelerate decomposition in the presence of the other constituents, and then gelatinizing the mixture. 10
12. A propellant explosive comprising a gelatinous admixture of nitrocellulose, nitro-glycerin, a non-volatile gelatinizing agent sufficiently soluble in the nitro-glycerin to remain dissolved in the mixture, and a stabilizing agent capable of taking up any products of decomposition, and which will not accelerate decomposition in the presence of the other constituents. 15
13. A propellant explosive comprising a gelatinous admixture of nitrocellulose, nitro-glycerin, a non-volatile aromatic gelatinizing compound sufficiently soluble in the nitro-glycerin to remain dissolved in the mixture, and a stabilizing agent capable of taking up any products of decomposition, and which will not accelerate decomposition in the presence of the other constituents. 20
14. A propellant explosive comprising a gelatinous admixture of nitrocellulose, nitro-glycerin, a non-volatile gelatinizing agent sufficiently soluble in the nitro-glycerin to remain dissolved in the mixture, and an aromatic stabilizing compound capable of taking up any products of decomposition, and which will not accelerate decomposition in the presence of the other constituents. 25
15. A propellant explosive comprising a gelatinous admixture of nitrocellulose, nitro-glycerin, a non-volatile aromatic gelatinizing compound sufficiently soluble in the nitro-glycerin to remain dissolved in the mixture, and an aromatic stabilizing compound capable of taking up any products of decomposition, and which will not accelerate decomposition in the presence of the other constituents. 30
16. A propellant explosive comprising a gelatinous admixture of nitrocellulose, nitro-glycerin, a non-volatile gelatinizing agent sufficiently soluble in the nitro-glycerin to remain dissolved in the mixture, and a stabilizing agent soluble in the mixture capable of taking up any products of decomposition, and which will not accelerate decomposition in the presence of the other constituents. 35
17. A propellant explosive comprising a gelatinous admixture of nitrocellulose, nitro-glycerin, a non-volatile aromatic gelatinizing compound sufficiently soluble in the nitro-glycerin to remain dissolved in the mixture, and a stabilizing agent soluble in the mixture capable of taking up any products of decomposition, and which will not accelerate decomposition in the presence of the other constituents. 40
18. A propellant explosive comprising a gelatinous admixture of nitrocellulose, nitro-glycerin, a non-volatile gelatinizing agent sufficiently soluble in the nitro-glycerin to remain dissolved in the mixture, and an aromatic stabilizing compound soluble in the mixture capable of taking up any products of decomposition, and which will not accelerate decomposition in the presence of the other constituents. 45
19. A propellant explosive comprising a gelatinous admixture of nitrocellulose, nitro-glycerin, a non-volatile aromatic gelatinizing compound sufficiently soluble in the nitro-glycerin to remain dissolved in the mixture, and an aromatic stabilizing compound soluble in the mixture capable of taking up any products of decomposition, and which will not accelerate decomposition in the presence of the other constituents. 50
20. A propellant explosive comprising a gelatinous admixture of a relatively large amount of nitrocellulose, a relatively large amount of nitro-glycerin, and relatively small amounts of a non-volatile substance capable of gelatinizing nitrocellulose and a non-volatile stabilizer capable of absorbing the products of slow decomposition of such nitric esters during storage, the admixed substances being soluble to such an extent in nitro-glycerin as to insure substantial homogeneity in the final explosive and being free from the property of accelerating decomposition of the constituents present. 55
21. A propellant explosive consisting of at least about 40 parts of nitroglycerin, relatively small amounts of a non-volatile substance capable of gelatinizing nitrocellulose and a non-volatile stabilizer capable of absorbing the products of slow decomposition of such nitric esters during storage, the balance of 100 parts being mainly nitrocellulose, the gelatinizer and stabilizer being soluble to such an extent in nitro-glycerin as to insure substantial homogeneity in the final explosive and free from the property of accelerating decomposition of the constituents present. 60
22. A propellant explosive comprising a gelatinous admixture of a relatively large amount of nitrocellulose, a relatively large amount of nitro-glycerin and relatively small amounts of a non-volatile substance capable of gelatinizing nitrocellulose and a non-volatile stabilizer capable of absorbing the products of slow decomposition of such nitric esters during storage, the gelatinizer and stabilizer being soluble to such an extent in nitro-glycerin as to insure substantial homogeneity in the final explosive and free from the property of accelerating the decomposition of the constituents present, 65

at least one of the two substances added in small amount being a readily nitratable aromatic-radical-containing compound.

23. A propellant explosive consisting of 5 at least about 40 parts of nitro-glycerin, relatively small amounts of a non-volatile substance capable of gelatinizing nitrocellulose and a non-volatile stabilizer capable of absorbing the products of slow decompo- 10 sition of such nitric esters during storage, the balance of 100 parts being mainly nitrocellulose, the gelatinizer and stabilizer being soluble to such an extent in nitro-glycerin as to insure substantial homogeneity 15 in the final explosive and free from the property of accelerating decomposition of the constituents present, at least one of the two substances added in small amount being a readily nitratable aromatic-radical- 20 containing compound.

24. A propellant explosive consisting of at least about 40 parts of nitro-glycerin, a non-volatile substance, capable of gelatinizing nitrocellulose and a non-volatile sta- 25 bilizer capable of absorbing the products of slow decomposition of such nitric esters during storage, the balance of 100 parts being mainly nitrocellulose, the gelatinizer and stabilizer being soluble to such an extent in 30 nitro-glycerin as to insure substantial homogeneity in the final explosive and free from the property of accelerating decomposition of the constituents present.

25. A propellant explosive consisting of

at least about 40 parts of nitro-glycerin, a 35 non-volatile substance, capable of gelatinizing nitrocellulose and a non-volatile sta- bilizer capable of absorbing the products of slow decomposition of such nitric esters during storage, the balance of 100 parts being 40 mainly nitrocellulose, the gelatinizer and stabilizer being soluble to such an extent in nitro-glycerin as to insure substantial homogeneity 45 in the final explosive and free from the property of accelerating decomposition 45 of the constituents present, at least one of the two last mentioned substances being a readily nitratable aromatic-radical-contain- ing compound.

26. A propellant explosive comprising a 50 gelatinous admixture of soluble nitrocellulose, nitro-glycerin, a gelatinizer and phe- nanthrene.

In testimony whereof we have signed our names to this specification in the presence of 55 two subscribing witnesses.

FREDERIC LEWIS NATHAN.  
WILLIAM RINTOUL.

Witnesses:

M. B. NICHOL,  
ALEX FORBES.

HENRY BAKER,  
*Administrator of the estate of Frank Baker,*  
deceased.

Witnesses:

P. A. OSMTHWAITE,  
BERTRAM H. MATTHEWS.